

**United States Patent** [19]  
**Sung**

[11] **Patent Number:** **4,869,728**  
[45] **Date of Patent:** **Sep. 26, 1989**

[54] **MOTOR FUEL ADDITIVE AND  
ORI-INHIBITED MOTOR FUEL  
COMPOSITION**

[75] Inventor: **Rodney L. Sung**, Fishkill, N.Y.

[73] Assignee: **Texaco Inc.**, White Plains, N.Y.

[21] Appl. No.: **245,591**

[22] Filed: **Sep. 19, 1988**

[51] Int. Cl.<sup>4</sup> ..... **C10L 1/18; C10L 1/22;**  
C07C 102/04

[52] U.S. Cl. .... **44/71; 44/73;**  
564/138; 564/141; 564/204; 564/208; 564/215

[58] **Field of Search** ..... **44/71, 73; 564/138,**  
564/141, 160, 193, 199, 204, 215, 208

[56] **References Cited**

**U.S. PATENT DOCUMENTS**

|           |        |             |         |
|-----------|--------|-------------|---------|
| 3,092,475 | 6/1963 | Cole et al. | 44/73   |
| 3,804,763 | 4/1974 | Meinhardt   | 44/71   |
| 3,806,456 | 4/1974 | Vogel       | 44/71   |
| 4,134,916 | 1/1979 | Moss et al. | 564/204 |

|           |         |                   |         |
|-----------|---------|-------------------|---------|
| 4,236,020 | 11/1980 | Lewis et al.      | 44/71   |
| 4,301,083 | 11/1981 | Yoshimura et al.  | 564/204 |
| 4,305,731 | 12/1981 | Sung et al.       | 44/63   |
| 4,394,493 | 7/1983  | Bartkovitz et al. | 564/204 |
| 4,526,587 | 7/1985  | Campbell          | 44/73   |
| 4,659,336 | 4/1987  | Sung et al.       | 44/71   |
| 4,659,337 | 4/1987  | Sung              | 44/71   |
| 4,695,291 | 9/1987  | Plavac            | 44/71   |
| 4,744,801 | 5/1988  | Taylor et al.     | 44/71   |

*Primary Examiner*—William R. Dixon, Jr.

*Assistant Examiner*—Ellen M. McAvoy

*Attorney, Agent, or Firm*—Robert A. Kulason; James J. O'Loughlin

[57] **ABSTRACT**

A motor fuel composition which inhibits engine ORI comprises a mixture of hydrocarbons boiling in the range of 90° F.-450° F. and the reaction product of one or more substituted or unsubstituted aliphatic carboxylic acids, including acyl-containing aliphatic carboxylic acids, and a polyoxyalkylene diamine.

**4 Claims, No Drawings**

## MOTOR FUEL ADDITIVE AND ORI-INHIBITED MOTOR FUEL COMPOSITION

### BACKGROUND OF THE INVENTION

#### 1. Field of the Invention

This invention relates to a novel reaction product composition and an ORI-inhibited motor fuel composition. More particularly, this invention relates to a reaction product composition obtained by reacting one or more aliphatic carboxylic acids and a polyoxyalkylene diamine, and an ORI-inhibited motor fuel composition containing such a reaction product.

#### 2. Information Disclosure Statement

Co-assigned U.S. patent application Ser. No. 07/239,865, filed Sept. 2, 1988 (D#78,507) discloses a motor fuel composition comprising the reaction product of one or more aliphatic carboxylic acids and a polyoxyalkylene diamine, the motor fuel composition having reduced engine ORI.

Co-assigned U.S. patent application Ser. No. 211,937, filed June 27, 1988 discloses a motor fuel composition comprising the reaction product of (i) a hydrocarbyl-substituted dibasic acid anhydride and (ii) a polyoxyalkylene diamine and an optional polymeric component which is a polyolefin polymer/copolymer, or mixtures thereof, of a C<sub>2</sub>-C<sub>10</sub> hydrocarbon.

Co-assigned U.S. patent application Ser. No. 84,354, filed Aug. 12, 1987 discloses a motor fuel composition comprising (I) the reaction product of the polyoxyalkylene diamine of co-assigned U.S. Pat. No. 4,747,851, a dibasic acid anhydride, and a hydrocarbyl polyamine, and (II) a mixture comprising polyisobutylene ethylene diamine and polyisobutylene in a hydrocarbon solvent.

Co-assigned U.S. patent application Ser. No. 000,230, filed Jan. 2, 1987 discloses a motor fuel composition comprising the reaction product of the polyoxyalkylene diamine of U.S. Pat. No. 4,747,851, a dibasic acid anhydride, and a hydrocarbyl polyamine. An optional additional polymer/copolymer additive with a molecular weight of 500-3500 may also be employed in conjunction with the reaction product additive.

Co-assigned U.S. Pat. No. 4,747,851 discloses a novel polyoxyalkylene diamine compound of the formula:



where c has a value from about 5-150, b+d has a value from about 15-150, and a+e has a value from about 2-12. Motor fuel compositions comprising the novel



polyoxyalkylene diamine, alone or in combination with a polymer/copolymer additive are also disclosed.

Co-assigned U.S. Pat. No. 4,659,337 discloses the use of the reaction product of maleic anhydride, a polyether polyamine containing oxyethylene and oxypropylene ether moieties, and a hydrocarbyl polyamine; and (ii) a polyolefin polymer/copolymer as an additive in motor fuel compositions to reduce engine ORI.

Co-assigned U.S. Pat. No. 4,659,336 discloses the use of the mixture of: (i) the reaction product of maleic anhydride, a polyether polyamine containing oxyethylene and oxypropylene ether moieties, and a hydrocarbyl polyamine; and (ii) a polyolefin polymer/copolymer as an additive in motor fuel compositions to reduce engine ORI.

U.S. Pat. No. 4,604,103 discloses a motor fuel deposit control additive for use in internal combustion engines which maintains cleanliness of the engine intake system without contributing to combustion chamber deposits or engine ORI. The additive disclosed is a hydrocarbyl polyoxyalkylene polyamine ethane of molecular weight range 300-2500 having the formula



where R is a hydrocarbyl radical of from 1 to about 30 carbon atoms; R' is selected from methyl and ethyl; x is an integer from 5 to 30; and R'' and R''' are independently selected from hydrogen and -(CH<sub>2</sub>CH<sub>2</sub>NH<sub>2</sub>)<sub>y</sub>-H where y is an integer from 0-5.

Co-assigned U.S. Pat. No. 4,758,247 discloses the use of the reaction product of an N-acyl sarcosine and a polyoxyalkylene polyol as a motor fuel additive in reducing engine deposit formation and engine ORI.

Co-assigned U.S. Pat. No. 4,305,731 (Sung et al.) discloses the use of the reaction product of an N-acyl sarcosine and a polyalkylene polyamine as a corrosion inhibiting additive in motor fuel compositions.

U.S. Pat. No. 4,198,306 (Lewis) discloses the use of hydrocarbyl poly (oxyalkylene) aminoesters which are monoesters of a hydrocarbyl-terminated poly (oxyalkylene) alcohol and a monocarboxylic C<sub>2</sub>-C<sub>20</sub> (amino-substituted) alcanoic acid as an ORI-controlling additive in motor fuel compositions.

### SUMMARY OF THE INVENTION

According to this invention, a novel reaction product which provides ORI-inhibiting properties to a motor fuel composition is obtained by reacting, at a temperature of 30° C.-200° C.:

(a) 0.5-2.5 moles of one or more aliphatic carboxylic

acids; and

(b) 0.5-1.5 moles of a polyoxyalkylene diamine of the formula



where R<sub>1</sub> and R<sub>2</sub> are C<sub>1</sub>-C<sub>12</sub> alkylene groups, q and r are integers having a value of 0 or 1, c has a value from 2-150, b+d has a value from 2-150, and a+e has a value from 0-12.

The motor fuel composition of the instant invention comprises a mixture of hydrocarbons boiling in the range of 90° F.-450° F. comprising from about

0.0005-5.0 wt. % of the abovedescribed reaction product.

### DETAILED EMBODIMENTS OF THE INVENTION

Combustion of a hydrocarbon motor fuel in an internal combustion engine generally results in the formation and accumulation of deposits on various parts of the combustion chamber as well as on the fuel intake and exhaust systems of the engine. The presence of deposits in the combustion chamber seriously reduces the operating efficiency of the engine. First, deposit accumulation within the combustion chamber inhibits heat transfer between the chamber and the engine cooling system. This leads to higher temperatures within the combustion chamber, resulting in increases in the end gas temperature of the incoming charge. Consequently, end gas auto-ignition occurs, which causes engine knock. In addition, the accumulation of deposits within the combustion chamber reduces the volume of the combustion zone, causing a higher than design compression ratio in the engine. This, in turn, also results in serious engine knocking. A knocking engine does not effectively utilize the energy of combustion. Moreover, a prolonged period of engine knocking will cause stress fatigue and wear in vital parts of the engine. The above-described phenomenon is characteristic of gasoline powered internal combustion engines. It is usually overcome by employing a higher octane gasoline for powering the engine, and hence has become known as the engine octane requirement increase (ORI) phenomenon. It would therefore be highly advantageous if engine ORI could be substantially reduced or eliminated by preventing or modifying deposit formation in the combustion chambers of the engine.

It is one object of this invention to provide a reaction product composition which may be employed as an ORI-reducing additive in motor fuel compositions. It is another object of this invention to provide a motor fuel composition which exhibits ORI-inhibition when employed in an internal combustion engine.

It is a feature of motor fuel compositions of the instant invention that combustion chamber deposit formation is minimized, with concomitant reduction of engine ORI.

It is an advantage that motor fuel compositions of the instant invention exhibit reduced engine ORI.

The ORI-inhibiting additive of the instant invention is a reaction product prepared by reacting one or more aliphatic carboxylic acids and a polyoxyalkylene diamine containing block copolymers with polyoxyalkylene backbones.

The aliphatic carboxylic acid reactant used to prepare the reaction product additive of the instant invention may be a saturated or unsaturated aliphatic carboxylic monocarboxylic acid. In one preferred embodiment of the instant invention, the aliphatic monocarboxylic acid reactant of the instant invention is an unsaturated aliphatic monocarboxylic acid selected from the group consisting of acrylic, propiolic, methacrylic, crotonic, isocrotonic, oleic, elaidic, maleic and fumaric acid, most preferably oleic acid.

In another preferred embodiment of the instant invention, the aliphatic monocarboxylic acid reactant is a saturated aliphatic monocarboxylic acid selected from the group consisting of formic, acetic, propionic, butyric, isobutyric, valeric, pivalic, lauric, myristic, palmitic, and stearic acid, most preferably palmitic acid.

In yetanother preferred embodiment of the instant invention, the aliphatic monocarboxylic acid reactant is one or more saturated aliphatic monocarboxylic acid of the formula



where n is an integer having a value of 0-5, x is an integer having a value of 0-10, X is H or a C<sub>1</sub>-C<sub>20</sub> alkyl group, and R<sub>3</sub>, R<sub>4</sub>, and R<sub>5</sub> are C<sub>2</sub>-C<sub>20</sub> alkyl groups. In one preferred embodiment, n is 0, x is 0, and R<sub>3</sub> and R<sub>5</sub> are —C<sub>14</sub>H<sub>29</sub>; therefore the aliphatic monocarboxylic acid reactant is of the formula



In another preferred embodiment, n is 2, X is H, x is 0, R<sub>3</sub> is —C<sub>14</sub>H<sub>29</sub> and R<sub>5</sub> is —C<sub>12</sub>H<sub>25</sub>; therefore the aliphatic monocarboxylic acid reactant is of the formula



In yet another preferred embodiment, n is 0, x has a value of 1-5, preferably about 5, X, R<sub>3</sub>, and R<sub>5</sub> are —C<sub>14</sub>H<sub>29</sub>, and R<sub>4</sub> is —C<sub>12</sub>H<sub>25</sub>; therefore the aliphatic monocarboxylic acid reactant is of the formula



In one particularly preferred embodiment of the instant invention, the abovedescribed aliphatic monocarboxylic acid reactant is a mixture of linear and telomer acids. A commercially available mixture of linear and telomer acids suitable for use as the aliphatic monocarboxylic acid reactant of the instant invention is available from Akzo Chemie B.V. under the KORTACID-T trade name. The most preferred KORTACID for use is KORTACID-T 1401, which comprises a mixture of

- (i) palmitic acid;
- (ii) acids of the formula



- (iii) acids of the formula



- (iv) acids of the formula



where  $x$  is an integer having a value of 1-5.

In yet another embodiment of the instant invention, the aliphatic monocarboxylic acid reactant is an acyl-containing aminocarboxylic acid of the formula



where R<sub>6</sub> is a C<sub>8</sub>–C<sub>24</sub> alkyl group, preferably a C<sub>12</sub>–C<sub>20</sub> alkyl group and R<sub>7</sub> is a C<sub>1</sub>–C<sub>6</sub> alkyl group, most preferably CH<sub>3</sub>. R<sub>6</sub> is most preferably an alkyl group selected from the group consisting of oleyl, coco, lauryl, tallow, and stearyl, and therefore in this embodiment the aliphatic carboxylic acid reactant is most preferably an acyl-containing aminocarboxylic acid selected from the group consisting of oleoyl, lauroyl, cocoyl, stearoyl, and talloyl sarcosine.

Examples of N-acyl sarcosine reactants suitable for use include talloyl sarcosine sold under the HAMPO-SYL-T trade name by W. R. Grace Company, as well as N-acyl sarcosines those sold under the SARKOSYL trademark by the Ciba-Geigy Company, such as SARKOSYL-O (oleoyl sarcosine) having a molecular weight in the range of about 345-360, SARKOSYL-L (lauroyl sarcosine), having a molecular weight in the range of about 270-285, SARKOSYL-LC (cocoyl sarcosine), having a molecular weight in the range of about 285-300, SARKOSYL-S (stearoyl sarcosine), having a molecular weight in the range of about 330-345, and SARKOSYL-T (talloyl sarcosine), having a molecular weight in the range of about 360-370. Talloyl and oleoyl sarcosine are particularly preferred for use as the N-acyl sarcosine reactants.

The polyoxyalkylene diamine reactant used to prepare the reaction product component of the instant invention is a diamine of the formula



where  $R_2$  and  $R_3$  are  $C_1-C_{12}$  alkylene groups, preferably  $C_2-C_6$  alkylene group, most preferably a propylene or butylene group,  $q$  and  $r$  are integers having a value of 0 or 1, preferably with  $q=1$  and  $r=0$ ,  $c$  has a value from about 2-150, preferably 2-50;  $b+d$  has a value from about 2-150, preferably 2-50; and  $a+e$  has a value from about 0-12, preferably 2-8. In one preferred embodiment,  $q=1$ ,  $r=0$ ,  $R_2$  is a butylene group and the polyoxoalkylene diamine reactant is therefore of the formula

where  $c$  has a value of from 2-150, preferably 2-50,  $b+d$  has a value of from 2-150, preferably 2-50 and  $a+e$  has a value of 2-12, preferably 2-8.

In another preferred embodiment,  $q=1$ ,  $r=0$ ,  $R_2$  is a propylene group,  $a+e$  has a value of zero, and the poly-oxyalkylene diamine reactant is therefore of the formula



where c and b+d, respectively, have a value of from 2-150, preferably 2-50. Polyoxyalkylene diamines of the above structure suitable for use include those available from Texaco Chemical Co. under the JEFFAMINE ED-Series trade name. Specific examples of such compounds are set forth below:

| Trade Name | Approx. Value |       | Approx.<br>Mol. Wt. |
|------------|---------------|-------|---------------------|
|            | c             | b + d |                     |
| ED-600     | 8.5           | 2.5   | 600                 |
| ED-900     | 15.5          | 2.5   | 900                 |
| ED-2001    | 40.5          | 2.5   | 2000                |
| ED-4000    | 86.0          | 2.5   | 4000                |
| ED-6000    | 131.5         | 2.5   | 6000                |

30 The reaction product component of the instant invention is prepared by reacting 0.5-2.5 moles, preferably about 2 moles of one or more aliphatic carboxylic acids with 0.5-1.5 moles, preferably 1 mole of the prescribed polyoxyalkylene diamine reactant, at a temperature of 30° C.-200° C., preferably 90° C.-150° C. until all of the water has been removed from the system. The reaction is 35 preferably carried out in the presence of a solvent. A preferred solvent is one which will distill with water azeotropically. Suitable solvents include hydrocarbons boiling in the gasoline boiling range of about 30° C. to about 200° C. Generally, this will include saturated and 40 unsaturated hydrocarbons having from about 5 to about 10 carbon atoms. Specific suitable hydrocarbon solvents include hexane, cyclohexane, benzene, toluene, and mixtures thereof. Xylene is the preferred solvent. The solvent can be present in an amount of up to about



90% by weight of the total reaction mixture. Once the reaction has been completed, the reaction product can then be separated from the solvent using conventional means, or left in admixture with some or all of the solvent.

The following examples illustrate the preferred method of preparing the reaction product of the instant invention. It will be understood that the following examples are merely illustrative, and are not meant to limit the invention in any way. In the examples, all parts are parts by weight unless otherwise specified.



## EXAMPLE I

C. until no more water can be removed from the system. The polyoxyalkylene diamine is of the formula



4.1 parts of oleic acid, 182.4 parts of xylene, and 168.3 parts of a polyoxyalkylene diamine were reacted at a temperature of about 90°-150° C. until no more water could be removed from the system. The polyoxyalkylene diamine (JEFFAMINE ED-2001) may be represented by the formula



there c has an approximate value of 40.5, and b+d has an approximate value of 2.5. The reaction product was then filtered and stripped of remaining solvent under vacuum, and identified by IR, NMR, and elemental analysis.

## EXAMPLE II

120 parts of a mixture of aliphatic monocarboxylic acids (KORTACID-T 1401), 500 parts of xylene, and 3366 parts of a polyoxyalkylene diamine were reacted at a temperature of about 90°-150° C. until no more water could be removed from the system. The polyoxyalkylene diamine (JEFFAMINE ED-2001) may be represented by the formula



where c has an approximate value of 40.5, and b+d has an approximate value of 2.5. The reaction product was then filtered and stripped of remaining solvent under vacuum, and identified by IR, NMR, and elemental analysis.

## EXAMPLE III

18.3 parts of talloyl sarcosine (HAMPOSYL-T), 186.6 parts of xylene, and 168.3 parts of a polyoxyalkylene diamine were reacted at a temperature of about 90°-150° C. until no more water could be removed from the system. The polyoxyalkylene diamine (JEFFAMINE ED-2001) may be represented by the formula



where c has an approximate value of 40.5, and b+d has an approximate value of 2.5. The reaction product was then filtered and stripped of remaining solvent under vacuum, and identified by IR, NMR, and elemental analysis.

## EXAMPLE IV

710 parts of oleoyl sarcosine (HAMPOSYL-O), 4000 parts of xylene, and 3366 parts of a polyoxyalkylene diamine are reacted at a temperature of about 90°-150°

15 where c has an approximate value of 40.5, b+d has an approximate value of 40.5, and a+e has an approximate value of 2.5.

The motor fuel composition of the instant invention comprises a major amount of a base motor fuel and 0.0005-5.0 weight percent, preferably 0.0001-1.0 20 weight percent of the abovedescribed reaction product. The fuel may also optionally comprise 0.001-1.0 weight percent, preferably 0.01-0.5 weight percent of the abovedescribed optional polymeric component. Preferred base motor fuel compositions are those intended 25 for use in spark ignition internal combustion engines. Such motor fuel compositions, generally referred to as gasoline base stocks, preferably comprise a mixture of hydrocarbons boiling in the gasoline boiling range, preferably from about 90° F. to about 450° F. This base 30 fuel may consist of straight chains or branched chains or paraffins, cycloparaffins, olefins, aromatic hydrocarbons, or mixtures thereof. The base fuel can be derived from, among others, straight run naphtha, polymer gasoline, natural gasoline, or from catalytically cracked 35 or thermally cracked hydrocarbons and catalytically reformed stock. The composition and octane level of the base fuel are not critical and any conventional motor fuel base can be employed in the practice of this invention. An example of a motor fuel composition of 40 the instant invention is set forth in Example V, below.

## EXAMPLE V

30 PTB of the reaction product set forth in Example I (i.e. 30 pounds of reaction product per 1000 barrels of 45 gasoline, equivalent to about 0.01 weight percent of reaction product based on the weight of the fuel composition) is blended with a major amount of a base motor fuel (herein designated as Base Fuel A) which is a premium grade gasoline essentially unleaded (less than 0.05 g of tetraethyl lead per gallon), comprising a mixture of hydrocarbons boiling in the gasoline boiling range consisting of about 22% aromatic hydrocarbons, 11% olefinic carbons, and 67% paraffinic hydrocarbons, boiling in the range from about 90° F. to 450° F.

55 The efficacy of the reaction product of the instant invention as an ORI-controlling additive in motor fuel compositions has been demonstrated by subjecting the reaction products exemplified by Examples I, II, and III, as well as two commercially available fuel additives 60 (OGA-480 and OGA-472, both available from Chevron Chemical Company) to Thermogravimetric Analysis (TGA). As discussed at Col. 12, lines 30-62 of U.S. Pat. No. 4,198,306 (Lewis), incorporated herein by reference, deposit control additives showing low TGA values, i.e. more rapid thermal decomposition, have been found to show low ORI values in laboratory engine tests. The results of the TGA tests are set forth below:

| Compound    | TGA Test Results                                 |  |
|-------------|--------------------------------------------------|--|
|             | Weight Remaining (%) after<br>30 min. at 295° C. |  |
| OGA-480     | 3.3                                              |  |
| OGA-472     | 64.4                                             |  |
| Example I   | 3.8                                              |  |
| Example II  | 18.7                                             |  |
| Example III | 23.7                                             |  |

It is well known to those skilled in the art that additive OGA-480 controls engine ORI but that OGA-472 tends to cause engine ORI. From the above TGA data, Example I has approximately the same % TGA residue as OGA-480, and therefore should have corresponding ORI-controlling properties. Examples II and III yielded % TGA residue values greater than OGA-480 but less than OGA-472, and therefore should have corresponding ORI-controlling properties greater than OGA-472 but less than OGA-480 and Example I.

For convenience in shipping and handling, it is useful to prepare a concentrate of the reaction product of the instant invention. The concentrate may be prepared in a suitable liquid solvent such as toluene or xylene, with xylene being particularly preferred.

In a preferred mode of preparing a concentrate of the instant invention, approximately 0.1-10.0, preferably 5.0-10.0 weight percent of the reaction product of the instant invention is blended with a major amount of liquid solvent, preferably xylene.

Motor fuel and concentrate compositions of the in-

descriptive terms and expressions, of excluding equivalents of the features described and it is recognized that various modifications are possible within the scope of the invention claimed.

The invention claimed is:

1. A composition obtained by reacting, at a temperature of 30° C.-200° C.:

(a) 0.5-2.5 moles of one or more aliphatic carboxylic acids selected from the group consisting of formic, acetic, propionic, butyric, isobutyric, valeric, pivalic, acrylic, propiolic, methacrylic, crotonic, isocrotonic, maleic and fumaric acid; and

(b) 0.5-1.5 moles of a polyoxyalkylene diamine of the formula



where  $\text{R}_1$  and  $\text{R}_2$  are  $\text{C}_1\text{-C}_{12}$  alkylene groups,  $q$  and  $r$  are integers having a value of 0 or 1,  $c$  has a value from 2-150,  $b+d$  has a value from 2-150, and  $a+e$  has a value from 0-12.

2. A composition according to claim 1, where said polyoxyalkylene diamine reactant is of the formula



where  $c$  has a value from about 2-50,  $b+d$  has a value from about 2-50, and  $a+e$  has a value from about 2-8.

3. A composition according to claim 1, where said polyoxyalkylene diamine reactant is of the formula



where  $c$  has a value of 2-50, and  $b+d$  has a value of 2-50.

4. A motor fuel composition comprising a mixture of hydrocarbons boiling in the range from about 90° F.-450° F. and additionally comprising from 0.0005-5.0 weight percent of the composition of any one of the preceding claims.

\* \* \* \* \*